

# United States Patent Office.

LOUIS CLOZEL, OF GRENOBLE, FRANCE.

Letters Patent No. 86,506, dated February 2, 1869.

## IMPROVED MODE OF TAWING SKINS OF ANIMALS.

The Schedule referred to in these Letters Patent and making part of the same.

To all to whom it may concern:

Be it known that I, LOUIS CLOZEL, of Grenoble, Isère, in the Empire of France, have invented a new and improved Mode of Tawing Skins of Animals; and I do hereby declare that the following is a full and exact description thereof.

In order to clearly show in what my invention consists, I will here explain the old method, viz:

The skins, after being steeped in pure water for several days, are plunged into a bath of lime, either pure, or mixed with a little sulphide of arsenic or orpiment, and, after remaining therein for some time, they are withdrawn in a condition for shaving or having the hair removed. After this latter operation, they are again subjected to a water-bath, in which they are turned about, so as to remove, as much as possible, all foreign-matter. It is necessary that the water for this purpose should be as pure as possible, and it is consequently frequently changed.

After the washing, the skins are placed in bran-baths, and after a time they are dressed, that is to say, they are steeped and stirred about in a mixture of water, corn, the yolk of eggs, alum, and sea-salt.

Having now described the old, I will proceed to mention the new system, the first modification in which consists in the employment of caustic potash or soda, sulphuret of sodium, or hypochlorite of potash or soda, known under the name of "eau de javelle," in place of the lime, for preparing the skins for the removal of the hair.

It is impossible to indicate the precise quantities of the ingredients alluded to, as they must necessarily vary according to the nature of the skins to be operated on; nevertheless, I commence always by putting the skins in a solution of one of these substances, in the proportion of one-tenth part to one hundred pints of water. The potash or soda which I prefer to employ is caustic, or I make use of a caustic solution of the before-mentioned substances, decarbonizing, by means of lime, a solution of carbonate of potash, soda, or sulphate of sodium, according to the quantity of lime employed, and in the proportions indicated by the law of chemical equivalents.

In the caustic solution thus formed, and deprived of the carbonates of lime, I plunge the skins; and although this solution is the best, it may be used without removing the carbonate of lime formed, or the excess of caustic lime. The skins, after remaining four or five days in this solution, are in a condition for having the hair removed. This is performed on leaving the solution, having previously plunged them in a simple water-bath, containing from one to three parts of sulphuric, nitric, chlorhydric, or acetic acid. This latter operation facilitates the removal of the hair.

The employment of these acids by manufacturing dressers, who make use of lime, would be of great importance. In this special case sulphuric acid must not be used, as the other acids form solubles with the de-

composed lime, and admit of the skins being more readily dressed when the hair is removed.

After leaving the last-named bath, they are plunged into baths containing animal or vegetable substances, capable of a rapid and specially putrid fermentation, but not alcoholic, acetic, or lactic.

I compose these baths of matters either in a state of putrefaction, or of animal or vegetable substances capable of rapidly becoming so. I generally make use of urine, either pure or mixed with water, according as I wish the putrefaction of the skins to take place more or less rapidly; or, instead of urine, I can employ meat, blood, or water used in hemp-retting. This decomposition is communicated to the skins, which renders them supple, the fatty matters saponifying by the action of ammoniacal salts, and the skins are more readily cleansed, the labor being considerably reduced.

When sufficiently cleansed and softened, I place them in a bran or other amylaceous bath, after which they are dressed, or, in lieu of the simple bran-bath, I can employ, in conjunction therewith, a solution of water and acetic acid.

The substitution of the caustic potash or soda, or of the substances already referred to, in place of the lime, is of the utmost importance, as, for example, the lime is almost insoluble, consequently its action is not uniform. Moreover, in saponifying the fatty matters of the skins, the lime forms lime-soaps, sterates, oleates, or margarates of lime, almost insoluble; therefore it is only by a mechanical action that these elements can be removed from the skins, and very frequently the lime remains, in form of caustic or carbonate of lime, which renders the skins brittle, uneven, and of a bad color.

The length of time the skins are kept in the lime greatly impairs them.

The substitution of the ingredients before alluded to in place of the lime is, therefore, of the greatest importance, whether as regards the rapidity of manufacture, or of the quality of the skin, and it enables me to plunge the skins, as soon as they are prepared, for the removal of the hair, into the putrid-fermentation baths, whereas, if the hair had been removed by lime, they could not have borne them without a too rapid change, as they would become eaten before they could be properly cleansed.

It is for this reason that the dressers are obliged to keep the skins in water, and in summer time it is necessary that the water should be as pure and changed as often as possible.

Having discovered that the skins treated by the old method, or water-bath system, do not retain their suppleness, unless by gentle fermentation, such fermentation being less active when the water is less frequently changed, I conceived the idea of employing liquid putrefaction-baths, acting in a regular and uniform manner on every part of the skin. By this means the fatty matters become saponified, and the soaps remain in solution in the baths, and the skins attain rapidly, and re-

tain, their suppleness after being dyed, and the foreign matter is removed from the skins by the fermentation, and the cleansing is effected more rapidly and with less trouble.

Amongst the advantages of my system over the old, I may mention the reduction in manual labor, and in the cost of the manufacture, the skins being more supple, and taking and retaining a brilliant dye. The time required for the manufacture is also reduced, whilst as regards the instruments and apparatus employed, they remain unchanged, as they are the same as those in present use.

What I claim as my invention, and desire to secure by Letters Patent, is—

The employment of caustic potash or soda solutions, or other substances, as hereinbefore explained, for removing the hair, and the use of the putrid-fermentation baths, not acid, as well as the bran-fermentation, specially acid.

L. CLOZEL.

Witnesses:

ALBERT I. DE ZEYK,  
T. F. GERVASY.